

Patented June 18, 1929.

1,717,800

# UNITED STATES PATENT OFFICE.

ROBERT A. MARR, OF NORFOLK, VIRGINIA.

## PROCESS OF TREATING CANE MATERIAL.

No Drawing.

Application filed October 17, 1922. Serial No. 595,215.

The present invention relates to the treatment of cane material, under which term is included various kinds of cane brake growth, such as *Machroasperma arundaria*, *Machroasperma tecta*, and various kinds of bamboo.

The invention embraces converting cane material of this character into various fibrous materials by treatment with a digestive solution, and subsequently working up 10 the material in any suitable manner, depending upon the final product which it is desired to obtain. The cane material may be treated either in a green or dry condition, and may be treated either in short or long 15 lengths depending upon the particular product which is desired, and the size and length of the material under treatment.

The cane, which may be cut up into suitable lengths and may be tied up into bundles 20 if desired, is placed into a solution preferably consisting of 1 part of zinc sulfate, 1 part of potassium sulfate, 2 parts of sodium sulfate. The said mixture being employed in amount equal to about 1½ to 2 ounces 25 of the mixture to each gallon of water. This forms a digestive solution of about 1 to 1½% strength, which is very much less concentrated than the usual digestive solutions heretofore generally used by others in making pulp. In the preferred form of carrying 30 out the process, the large cane cut into suitable lengths is placed into a digester (preferably in the form of bundles), the digester being packed as full as possible with 35 the bundles of material. The digester is then filled with the liquor above referred to, which may be cold or warm or even hot, and the cover is then placed on the digester in an air tight manner. The material is then 40 cooked by heating the liquor in any suitable manner, for example, by blowing in steam. The length of time and temperature of the cooking operation, will determine the degree 45 to which the cane material will be modified by the cooking operation.

For making fiber materials for stiff brushes and the like, the liquor will be heated up to a pressure of, for example, 75 pounds, this pressure being maintained for 50 15 or 20 minutes, after which the liquid may be allowed to cool sufficiently to bring the pressure back to about atmospheric, after which the cooked material may be removed from the hot liquor. For making materials 55 for spinning fibers, burlap, gunny cloth,

rope, twine and cordage, it is advisable to hold a pressure of about 100 pounds for 30 minutes or so. For making finer cloth, a pressure of 100 pounds, maintained for 30 to 40 minutes generally gives good results. 60

For making pulp for use in the manufacture of paper, plastic materials, such as artificial lumber or the like, the cane material may be heated in the solution up to a pressure of 140 pounds, which pressure may be 65 maintained for 1½ to 3 hours. It is to be understood that these pressures and temperature are given for the purpose of illustration and not as limiting the invention thereto. In all of the cases above mentioned, the digester with the solution and 70 cooked material can then be allowed to cool off somewhat, say until the pressure has dropped to about atmospheric and the temperature has dropped to somewhat below the 75 boiling point, after which the liquor can be drawn off from the digester or the bundles of material can be taken out of the digester leaving the liquor therein. The bundles of cooked material may be soaked in water at 80 ordinary temperature or hot water for ½ hour or so to remove any adhering chemicals. For making pulp from the cooked material, it can first be run through rollers 85 lengthwise of the grain, which will cause the same to be broken up into fiber bundles, which can then be run through a pulper and then through a Jordan engine. The material may then be made into sheets in the 90 usual manner. In place of using the Jordan, an ordinary beater engine can be used, if desired, this ordinarily not being necessary. A paper is produced in this manner 95 which is of a brownish color and is very strong, being stronger than many of the varieties of kraft paper. For making spinning fibers, ropes, gunny cloth and the like, it is advisable to add, directly after cooking and washing, an oleaginous material, such as an emulsion of oil (e. g. mineral oil) 100 and soap, as a lubricant. This serves as a conditioning material, and the oil employed may be mineral oil, fatty oil, or tar oil. The material is then run through rolls, which may be of hard material such as iron, or 105 wood, or of soft yielding material such as rubber. If the rolls are made of hard material they should not be pressed together too hard, since the strength of the fiber is liable to be injured if too much pressure is 110

used. If desired a device similar to an ordinary laundry clothes-wringer may be used in this operation. In case wooden or iron rolls are used it may be advisable to combine the oiling operation with the pressing operation, by allowing the bottom roll to dip into an oily material or an emulsion of an oily material. The rolled material can then run through a picker and a carding device and then may be used as a substitute for coir or cocoa fiber for making mats and matting or for making the coarse fabrics above referred to. Any of the waste from this operation may, if desired, be run through a pulper and can thereafter be used for making paper.

For working up the material above referred to for making brush or broom fiber, the cooked material may be washed and treated with an oily material as above referred to after which it can be passed through rolls in the manner above referred to. The material can then be brushed or carded for removing tow as a by-product, which tow can be worked up into fabrics, rope or pulp as above described.

When it is desired to produce very coarse bristles such as are used for brooms for street sweeping and the like, the cooked material, preferably after oiling, can be passed lengthwise through cutters spaced to produce the desired thickness.

The fiber either in the form of pulp, textile fiber or broom fiber or finished products containing these, may, if desired, be dyed by treatment with cotton dyes and alum, or other mordant.

Fiber made for brooms and brushes and also fiber made for bagging, ropes, cordage and the like can be water-proofed if desired. A suitable solution for this operation when prepared by dissolving lead acetate in water and separately therefrom dissolving alum or aluminum sulfate in water, adding agar agar to each of said solutions and mixing the same.

Another suitable mixture for making the material water-resistant is one consisting of lead acetate solution and a solution of copperas each containing gum or dextrin the two solutions being mixed together.

It is important to note that when using the small cane, particularly tecta, this material may be put into the digester without being cut into lengths, simply being bundled into large bundles to completely fill the digester or being made into small bundles which are then packed into the digester. These bundles are then cooked and on being run through rollers, the material breaks up at the joints or nodes, leaving the fiber material for further treatment.

In treating large cane and bamboo for making fiber, the cane may be cut into sections, cutting out the joints or nodes, then making bundles of substantially uniform

lengths of the cane material, preferably splitting up the same into several pieces. The nodes or joints which are thereby cut out can be cooked separately for the making of pulp so that it is not necessary to waste any of this material.

The digestive liquor above referred to is capable of being modified to some extent. The proportions of the materials as given above are those which have been found to give very satisfactory results. However, good results can be secured even when omitting the potassium sulfate and in a few cases good results have been secured when using a solution of sodium sulfate and potassium sulfate in about the ratio above referred to, this being used in the amount of about 2½ ounces per gallon of liquor. The particular preferred cooking liquor above referred to is especially advantageous in that it can be used over several times in the cooking of successive batches of the cane and it is not necessary to throw away the liquor and to make up fresh liquor after each cooking operation. I have repeatedly used the same liquor in more than a dozen successive cooks with satisfactory results.

The cooked material may take out a small quantity of the sulfates, and a portion of the water in the cooking liquor may be lost by evaporation owing to the high temperature used. The water in which the cooked material is soaked (and it may be noted that the time of soaking above given is merely by way of example) can be used in making up fresh quantities of liquor or can be used for making up any loss of liquor from the above solution. Further quantities of the sulfates referred to can be added from time to time to prevent the liquid from becoming unduly weakened by absorption. The liquid pressed out from the cooked material during the pressing operation above referred to likewise can be used for making up additional cooking liquid.

I claim:

1. A process of treating cane material of the character set forth which comprises digesting the same in a solution containing an alkali metal sulfate and zinc sulfate.

2. A process of treating cane material of the character set forth which comprises digesting the same in a solution containing an alkali metal sulfate and zinc sulfate, and carrying the pressure up to at least 75 pounds, for not less than 15 minutes.

3. A process of treating cane material of the character set forth which comprises digesting the same in a solution containing an alkali metal sulfate and zinc sulfate, and carrying the pressure up to at least 100 pounds for not less than 30 minutes.

4. A process of treating cane material of the character set forth which comprises digesting the same in a solution containing an

alkali metal sulfate and zinc sulfate, and carrying the pressure up to about 140 pounds for about 90 to 180 minutes.

5. A process of treating cane material of the character set forth which comprises digesting the same in a solution containing sodium sulfate, potassium sulfate and zinc sulfate.

10. A process of treating cane material of the character set forth which comprises digesting the same in a solution containing an alkali metal sulfate and zinc sulfate, and thereafter running the cooked material through pressure rolls.

15. 7. A process of treating cane material of the character set forth which comprises digesting the same in a solution containing an alkali metal sulfate and zinc sulfate, running the cooled material through pressure rolls and applying an oleaginous material thereto, the last-mentioned two steps being in any desired order.

8. A process of treating cane material of the character set forth which comprises digesting the same in a solution containing a plurality of alkali metal sulfate solutions.

25. 9. A process of treating cane material which comprises digesting the same in a sulfate solution containing an alkali metal sulfate 30 under pressure above atmospheric, and thereafter crushing said material.

30. 10. A process which comprises digesting cane material with a solution containing a plurality of sulfates including zinc sulfate

and thereafter reducing the size of the pieces 35 by mechanical treatment.

11. A process which comprises digesting cane material in a solution containing zinc sulfate and an alkali metal sulfate, such solution containing substantially less than 5% 40 of dissolved salts.

12. A process which comprises digesting cane material in a solution containing zinc sulfate and an alkali metal sulfate, such solution containing about 1 to 2% of said salts, 45 and being free from other strong added chemicals.

13. A process of treating cane material which comprises digesting the same in a solution containing an alkali metal salt and a 50 soluble salt of another metal, such solution being of about 1% to 2% strength, and repeatedly using the same digesting solution with a plurality of batches of the said cane material. 55

14. A process of treating cellulosic and ligneous material which comprises digesting the same in a sulfate solution containing an alkali metal sulfate and a soluble earth metal sulfate, together amounting to not over 2%, 60 such salts being the principal dissolved active constituents of such solution, such digestion being conducted under superatmospheric pressure, and repeatedly using the same digestive solution with a plurality of batches 65 of the said cellulosic and ligneous material.

In testimony whereof I affix my signature.  
ROBERT A. MARR.